

March 7, 1933.

C. A. COLOMBO

1,900,635

PROCESS FOR PRINTING TRANSFERS

Filed April 27, 1931



Inventor  
Carlo A. Colombo  
By Sommers, Young Atts

## UNITED STATES PATENT OFFICE

CARLO ALBINI COLOMBO, OF MILAN, ITALY, ASSIGNOR TO SOC. ITAL. TRANSFERS ALBINI,  
S. I. T. A., OF MILAN, ITALY

## PROCESS FOR PRINTING TRANSFERS

Application filed April 27, 1931, Serial No. 533,366, and in Italy April 29.

This invention relates to transfers which can be placed upon the surface of any porous material, such as e. g. wood, leather, wool, silk or cotton fabrics, sacks and bags, 5 etc.

The transfer prepared by the process according to this invention keeps for a very long time and can be placed at any moment upon a porous surface by the combined action of pressure and heat. 10

The colours of the transfer penetrate deeply into the porous surface giving at the same time a clear design without spreading.

The preparation or printing of the transfers is effected by means of lithographic and typographic machines on any paper either prepared or not. 15

The preparation of the inks or colours necessary for printing is effected as follows:

I melt in a suitable container 100 parts 20 of tallow and 100 parts of colophony, preferably of best quality. The word "tallow" as used throughout the specification and claims refers to the common meaning of the word, namely the tallow obtained from animals such as cattle, sheep and the like. The quantity of colophony employed varies according to the period of the year, i. e. I employ a larger quantity in the warm months 25 than in the colder ones. I thus obtain a sufficiently thick mass which can, however, be thinned like normal lithographic colours. The density of this paste can be reduced, if necessary, by the addition of one or more 30 parts of wax and one or more parts of glucose, without, however, exceeding a limit as would prevent a satisfactory printing. The mass thus obtained is mixed with any suitable lithographic ink in variable proportions 35 according to the density of the colour to be obtained, and the ink resulting therefrom will give most satisfactory results. 40

A similar result can be obtained by melting the colours with the mass during the preparation of this latter, whereby the colour ready for printing is obtained. 45

After having prepared the ink or printing colour on the palette in the manner above described, before introducing it into the ink 50 reservoir of the printing machine, it is ad-

visable to incorporate with the colour a sufficient quantity of colophony or other gum which has been previously finely ground, as the print will be more brilliant and clear. The ink acquires a granular aspect and the 55 print will be sticky.

A still better result is obtained, by dusting over the impression, immediately after print, with powdered colophony or other finely ground resinous gum. 60

The transfers thus obtained can be placed in an indelible manner upon a porous surface, on which the impression will be perfectly clear, brilliant and well-outlined.

The transfers according to this invention 65 do not stiffen the fabric on which they are placed and do not crack.

According to this invention the impression is conveniently transferred by rolling between two rolls the surface on which the impression is to be placed against the transfer, one of said rolls being driven while the other is loose and pressed against the former and heated by suitable means. 70

The annexed drawing shows one way of 75 carrying out the invention.

Referring to the drawing, 1 denotes the support of paper and 2 the layer representing the design or the like obtained by lithographic printing using the ink prepared as 80 above described.

What I claim is:

Process for preparing transfers adapted to be placed upon porous material, consisting in melting together tallow and colophony in equal parts, in adding to the mass resulting therefrom wax and glucose in order to obtain the desired density, in adding said mass to a lithographic colour in the desired proportions for obtaining the desired colour density and in printing the inscriptions and designs to be transferred on a sheet of paper by means of the ink prepared as above. 85

In testimony that I claim the foregoing 90 as my invention, I have signed my name.

CARLO ALBINI COLOMBO. 95